

## UNITED STATES PATENT OFFICE

2,303,363

PROCESS FOR RENDERING TEXTILES  
WATER-REPELLENT AND PRODUCT  
THEREFROMWalther Kaase and Ernst Waltmann, Kre-  
feld, Germany, assignors to Heberlein  
Patent Corporation, New York, N. Y., a cor-  
poration of New YorkNo Drawing. Application April 28, 1936, Serial  
No. 76,738. In Germany May 2, 1935

15 Claims. (Cl. 8—120)

This invention relates to processes for producing water-repellent fibrous materials and products therefrom.

It has been suggested heretofore that water-repellence be produced in cellulose-containing materials by treatment with esterifying agents such as fatty acid chlorides or fatty acid anhydrides. In the execution of these processes, however, difficulties have been encountered due to unfavorable reaction conditions whereby the appearance and feel of the goods is changed. These processes also require considerable time and expense for operation. The treatment of the material to render it water-repellent or drop-proof is carried out ordinarily as the final treatment in finishing the material. It is accordingly necessary from the standpoint of practical mass production that the process be carried out with considerable rapidity and be accomplished in a short period instead of requiring hours as heretofore.

The principal object of the present invention is to provide a simple process to increase water-resistance in materials, such as, for example, but without limitation, cotton, jute, linen, hemp and various artificial silks and wool, in a relatively short time and with less expense than that of the chlorides and anhydrides mentioned above; and to produce materials having improved characteristics.

The invention accordingly comprises the novel products as well as the novel processes and steps of processes according to which such products are manufactured, the specific embodiments of which are described hereinafter by way of example and in accordance with which we now prefer to practice the invention.

Now we have found in accordance with our invention that treatment of textile materials, including cellulose-containing materials and wool, with the extremely reactive isocyanic acid esters of the aliphatic, mixed aliphatic-aromatic or naphthenic series produces remarkably fine effects, including resistance to wetting by water. For this purpose only the isocyanic acid esters of the series mentioned having at least 10 carbon atoms for instance decylisocyanate, hexadecylisocyanate, heptadecylisocyanate, heneicosylisocyanate, octadecylisocyanate, docosylisocyanate etc. are to be employed. These substances may be prepared by well-known processes such as described in Berichte der Deutschen Chemischen Gesellschaft, 42d year, 1909, vol. 3 page 3359, cf. the article by Schroeter, "Ueber Umlagerungen." In the appended claims, cer-

tain of these isocyanates have been designated by the formula  $RN=C=O$ , where R is an aliphatic radical containing more than 10 carbon atoms. There are suitable also other isocyanates 5 which are obtained by transposition of saturated amines or mixtures of such saturated amines of high molecular weight with phosgene. Such amines of high molecular weight are commercially obtainable in the way described in German Patent No. 611,924 or French Patent No. 761,952.

This transposition is effected as follows: The 15 amine, for example stearylamine is dissolved in hot toluene, the solution is saturated with gaseous hydrochloric acid, whereby stearylamine hydrochloride separates out; then phosgene is passed into the mixture until solution occurs. The reactions which occur appear to be as follows:



It is not necessary to use pure saturated amines 25 as mixtures of saturated amines of high molecular weight are well suitable, for instance the mixture of amines which is obtained by hydrating train oil (whale oil) fatty acids.

Amines of high molecular weight such as described in British Patent No. 384,314 are also 30 capable of undergoing this transposition, for instance 18-amino-pentatriacontane yields 18-pentatriacontane isocyanate,  $C_{35}H_{71}NCO$ .

In addition to the isocyanates described above 35 the corresponding isocyanic acid esters of the naphthenic acids having at least 10 carbon atoms in an aliphatic portion are also suitable, for example a naphthenic acid from Galician naphtha corresponding to the formula:



or a bicyclic naphthenic acid  $C_{20}H_{37}COOH$  derived from Roumanian naphtha.

There may also be employed the isocyanate obtainable from montanic acid. Montanic or heptacosyl acid which corresponds to the formula:  $C_{27}H_{55}COOH$ , is converted into heptacosyl isocyanate in the usual way:



The statement above made that the aliphatic, mixed aliphatic-aromatic or naphthenic acids which form part of the esters should have at least 10 carbon atoms, means that there should

be at least 10 carbon atoms in the aliphatic portions of such esters. From ten carbon atoms upwards representing an even number or an uneven number of carbon atoms may be so present.

There may also be employed substances which are easily converted into the isocyanic acid esters upon treating the textiles herein mentioned with such substances under reaction conditions. For example we may employ the corresponding fatty acid azides such as palmitic acid azide



These substances become converted with elimination of nitrogen into the corresponding isocyanic acid esters, as described in "Journal für praktische Chemie" (2) vol. 64, page 430, cf. the article by Curtius Dellschafft.

Fatty acid azides occur as intermediate products if the way of preparing fatty acid chlorides and treating same with sodium azide is adopted, as is shown in the reactions on the preceding page of this specification. Furthermore fatty acid azides may be obtained, as is well known, by treating fatty acid hydrazides with nitrous acid  $\text{HNO}_2$ .

In accordance with our invention it has further been found that there may also be employed aliphatic isocyanates whose carbon chains are interrupted by the atoms or atomic groups O, S, N, CO.O, O.CO, NR', NR'.CO, CO.NR', SO<sub>2</sub>, NR'.SO<sub>2</sub>, SO<sub>2</sub>.NR' in which R' may be equal to hydrogen or may be any desired hydrocarbon radical (cf. French Patent No. 787,785). It is known that all carboxylic acid chlorides are easily converted into the corresponding azides and isocyanates by the Curtius method.

For the same purpose mixed aliphatic-aromatic isocyanic acid esters may also be used, in so far as they contain a saturated aliphatic radical of at least 10 carbon atoms. The active  $-\text{N}=\text{C}=\text{O}$  group may in this connection be tied directly to the aromatic ring, i. e., for example



which is 1-stearyl-oxy-phenylene-4-isocyanate. The aromatic radical may be hydrogenated, chlorinated, or otherwise replaced, and the hydrogenated compound, for example, may be represented by the formula



which is 4-carboctadecoxy tetrahydrophenyl isocyanate.

It is also possible to successfully use for water-repellence, isocyanates which contain in the alkyl radical the radical of a saturated or unsaturated alcohol of the sterol series. As a technological starting material for the alcohol of the sterol series there is advantageously employed the sterol mixtures contained in the unsaponifiable part of wool fat. Such mixtures may be prepared for instance in the manner described in German Patent No. 617,975. For the purpose of introduction of the active  $-\text{N}=\text{C}=\text{O}$  group these alcohols are converted into ester- or ether-carboxylic acids and the chlorides of these ester- or ether-carboxylic acids are converted by the Curtius method. Thus for example cholesterol which is an alcohol,



occurring in the unsaponifiable part of wool fat is transposed by means of adipic acid chloride according to the following reaction:



10 whereby cholesterol-adipic acid ester isocyanate is formed.

The new substances mentioned are distinguished by an extremely high rapidity of action towards textile materials, particularly towards cellulose and cellulose derivatives, such as has not heretofore been observed in connection with any of the known methods. It is necessary only to bring the textile material in contact with the isocyanate, as by passing the textile material briefly through a solution of the isocyanic acid esters in benzene or a suitable solvent and immediately thereafter it is subjected for several minutes to a high temperature to produce water-repellence.

15 25 An action between the textile material and the treating substance occurs in accordance with our invention to produce water-repellence but we do not wish to be understood to state unqualifiedly that a chemical reaction occurs between the textile material and the chemical compound employed in accordance with the invention, as we are not sure that such is the case.

30 One may also treat the fibers of cellulose or cellulose derivatives immediately after the spinning process with the esters herein mentioned, to obtain water-repellence.

35 Impregnation of the textile materials with the esters herein mentioned may be carried out in any desired manner with or without the use of organic solvents or of aqueous emulsions of the esters applied by soaking, spraying or the like. The addition of catalytic agents for the purpose of securing the desired effect may be made, but it is not necessary.

40 45 The water-repellent effect produced in accordance with our invention resists domestic washing. After thorough rinsing out of the soap employed for this purpose and drying, the textile material again manifests water-repellent properties. It is also resistant to dry cleaning.

50 55 The following are examples of embodiments of the invention as we now prefer to carry it out. It is to be understood that these examples are not to be construed as limiting the invention, except as indicated in the appended claims.

#### Examples

1. A printed crepe, having delustered viscose rayon as warp and viscose crepe as weft, is 60 passed through a 0.5% solution of octadecyl isocyanate,  $\text{C}_{18}\text{H}_{37}\text{N}=\text{C}=\text{O}$  in benzene. The time of passage is about 3 seconds and the solution is at room temperature. Immediately thereafter the so-treated material is subjected for one minute to a temperature of 100° C. (212° F.) and then for two minutes to a temperature of 140° C. (284° F.).

2. Acetate satin having acetate silk as warp and viscose crepe as weft is sprayed with a 1% 70 solution of heptacosyl (or montanyl) isocyanate,  $\text{C}_{27}\text{H}_{55}\text{N}=\text{C}=\text{O}$ , in benzene at room temperature. The solvent is evaporated off, and the so-treated material is subjected for two minutes to a temperature of 130° C.

75 3. Dyed stockings of Bemberg silk (cupram-

monium silk) are immersed in a 0.3% solution of heneicosylisocyanate  $C_{21}H_{43}N=C=O$ , in benzine at room temperature for approximately 10 seconds, then taken out and, after evaporation of the solvent, treated for 1½ minutes at 150° C.

4. A cotton tent cloth is passed through a 1% solution of naphthenic isocyanate,



in benzine. After the passage which lasts about 4 seconds, the solvent is evaporated off and the material is heated for 2 minutes to a temperature of 150° C.

5. A fabric, suitable for rucksacks, consisting of linen and cotton is treated with a 0.75% solution of bicyclic naphthen isocyanate,



from Roumanian naphtha in benzine in the same way as described in Example 4.

6. A viscose spun rayon fabric is treated with an 0.5% solution in benzine of 1-stearyl-oxy-phenylene-4-isocyanate,



in the same way as in Example 1.

7. A poplin from mercerized cotton, suitable for rain-proof overcoats is passed through a 0.5% solution of octacosan-acid azide in benzine. The solvent is then removed by heating the fabric to about 100° C. for a short time. Afterwards the material is exposed for two minutes to a temperature of 140°.

8. A mixture of amines obtainable by hydrating train oil acids (see page 1) is converted into a mixture of isocyanic esters by means of phosgene as above described and a 0.5% solution in benzine therefrom is prepared. A mixed fabric consisting of mercerized cotton and viscose spun rayon is treated with this solution in the same way as described in Example 7.

9. A fabric consisting of "Vistra" (spun viscose rayon) is treated with a 0.5% solution of cholesterol-adipic acid ester isocyanate.



in benzine as described in Example 7.

10. A wool muslin is treated with a 0.5% solution of cholesterol-adipic acid ester azide in benzine (see page 2),  $C_{27}H_{45}O.CO(CH_2)_4CON_3$ , as described in Example 7.

11. A worsted fabric is treated with a 0.5% solution of octacosan acid azide in benzine as described in Example 7.

12. A strong cotton fabric is passed during 3 seconds through a 0.5% solution of heptacosyl (montanyl) isocyanate,  $C_{27}H_{55}N=C=O$ , in benzine, the solvent is evaporated off and the material is exposed for 2 minutes to a temperature of 150° C.

The amount of the ester deposited in all of the above examples on the materials will naturally vary with the weight of the material. We have found that ordinarily an amount of the ester equal to about 0.5% of the material being treated, is sufficient to give the effect.

The materials produced in accordance with the above examples show a high degree of water-repellence. They show a lesser absorption of moisture as compared with the known processes employing fatty acid chlorides and fatty acid anhydrides. They show also greatly improved durability toward dry-cleaning, soap washing, etc. as compared with these previous materials. The feel and hang of the materials having water-repellence as produced above, is about the same

as that of the untreated material. Rayons especially, when treated in accordance with the invention, show an increase in tensile strength.

The process of the invention, particularly as set forth in the specific embodiments above, may be carried out with simple apparatus at relatively small expense and in a relatively short time.

In the claims and elsewhere where the expression "cellulose-containing material" is employed, it is intended to cover fibers, yarns, fabrics or other forms of cotton, jute, linen, hemp or rayon including viscose, cuprammonium, or other precipitated cellulose or derivatives of cellulose such as acetyl cellulose. Similarly, the expression "textile material" is intended to include such "cellulose-containing material" and similar forms of wool or other animal material.

The expression "isocyanate," as used in the claims, is intended to include not only isocyanates but also azides which are capable of liberating nitrogen to produce isocyanates and when applied to textiles and heated, for example, above 100° C. will act thereon to produce water-repellence therein.

Subject matter not herein claimed is claimed in our copending applications Serial No. 196,622, filed March 18, 1938, and Serial No. 221,994, filed July 29, 1938.

While the invention has been described in detail according to the preferred manner of carrying out the process, it will be obvious to those skilled in the art after understanding the invention, that changes and modifications may be made therein without departing from the spirit or scope of the invention, and it is intended in the appended claims to cover all such changes and modifications.

What is claimed as new and desired to be secured by Letters Patent, is:

1. A process for ennobling textile material which comprises subjecting the material to an isocyanate of the group consisting of aliphatic isocyanates, mixed aliphatic-aromatic isocyanates, and naphthenic isocyanates, which contain an aliphatic radical of at least 10 carbon atoms, and heating the material with the isocyanate to increase the water-repellence of said material.

2. A process for ennobling textile material which comprises subjecting the material to a naphthenic isocyanate having a naphthene radical containing an aliphatic radical of at least 10 carbon atoms, and heating the material with the isocyanate to increase the water-repellence of said material.

3. A process for ennobling textile material which comprises impregnating the material with an isocyanate of the group consisting of aliphatic isocyanates, mixed aliphatic-aromatic isocyanates, and naphthenic isocyanates, which contain an aliphatic radical of at least 10 carbon atoms, and heating the impregnated material for a short period at a temperature above 100° C. to increase the water-repellence of said material.

4. A process for ennobling artificial silk which comprises heating the artificial silk with an isocyanate of the group consisting of aliphatic isocyanates, mixed aliphatic-aromatic isocyanates, and naphthenic isocyanates, which contain an aliphatic radical of at least 10 carbon atoms capable of acting upon said material, for a short period at a temperature above 100° C., to increase the water-repellence of said silk.

5. A process for ennobling textile material

which comprises heating the material with an aliphatic-aromatic isocyanate, which contains a saturated aliphatic radical of at least 10 carbon atoms, the isocyanate group  $N=C=O$  being joined directly to the aromatic ring, to increase the water-repellence of said material.

6. A textile material heated with an isocyanate to render it water-repellent, said isocyanate being selected from the group consisting of aliphatic, mixed aliphatic-aromatic and naphthenic isocyanates, containing an aliphatic radical of at least 10 carbon atoms, said material having a water-repellent property but in appearance and feel being substantially the same as similar material untreated.

7. A textile material heated with an aliphatic isocyanate which contains an alkyl radical of at least ten carbon atoms, said material having a water-repellent property but in appearance and feel being substantially the same as similar material untreated.

8. A textile material heated with a naphthenic isocyanate having a naphthene radical containing an aliphatic radical of at least ten carbon atoms, said material having a water-repellent property but in appearance and feel being substantially the same as similar material untreated.

9. A textile material heated with an aliphatic-aromatic isocyanate which contains a saturated aliphatic radical of at least ten carbon atoms, said material having a water-repellent property but in appearance and feel being substantially the same as similar material untreated.

10. A process for treating textile material which comprises impregnating the material with an isocyanate of the formula  $RNCO$  in which  $R$  is an

5 aliphatic radical containing more than 10 carbon atoms, said isocyanate being capable of acting upon said textile material to render the same water-repellent, and heating the impregnated material to produce water-repellence therein.

11. A process for treating textile material which comprises impregnating the material with a isocyanate containing an aliphatic radical of at least ten carbon atoms capable of acting upon 10 said textile material to render the same water repellent, and heating the impregnated material to produce water-repellence therein.

12. A process for treating textile material which comprises impregnating the material with mixed aliphatic-aromatic isocyanate containing an aliphatic radical of more than 10 carbon atoms, and capable of acting upon said textile material to render the same water-repellent, and heating the impregnated material to produce water-repellence therein.

13. A process for treating textile material which comprises impregnating the material with mor tanyl isocyanate and heating the so impregnate material to render the same water-repellent.

14. A process for treating textile material which comprises impregnating the material with 1- $\alpha$  aryl-oxy-phenylene-4-isocyanate and heating the so impregnated material to render the same water-repellent.

15. A process for treating textile material which comprises impregnating the material with naphthenic isocyanate having the formula  $C_{10}H_{19}N=C=O$  and heating the so impregnate material to render the same water-repellent.

WALTHER KAASE.  
ERNST WALTMAN.

CERTIFICATE OF CORRECTION.

Patent No. 2,303,363.

December 1, 1942.

WALTHER KAASE, ET AL.

It is hereby certified that error appears in the printed specification of the above numbered patent requiring correction as follows: Page 2, second column, line 5, for that portion of the formula reading " $(CH_2)COCl + HCl$ " read  $--(CH_2)_4COCl + HCl--$ ; and that the said Letters Patent should be read with this correction therein that the same may conform to the record of the case in the Patent Office.

Signed and sealed this 2nd day of February, A. D. 1943.

(Seal)

Henry Van Arsdale,  
Acting Commissioner of Patents.